

## UNITED STATES PATENT OFFICE

2,262,778

DETERMINING THE IDENTITIES OF PIECES  
OF DIFFERENT STEELS

Herbert H. Schneider, East Cleveland, Ohio, assignor to The American Steel and Wire Company of New Jersey, a corporation of New Jersey

No Drawing. Application March 20, 1939,  
Serial No. 263,058

2 Claims. (Cl. 73—51)

This invention is concerned with the problem of economically and rapidly determining the identities of pieces of steels having different critical temperatures. Those in charge of the stock in a steel mill encounter this problem when different steels become mixed. At present the only solution is to chemically analyze each piece of steel, this being both expensive and slow.

The problem is particularly acute when stocks of SAE 1035 and SAE 1335 steels become mixed. Therefore, the principles of the invention are hereinafter discussed as applied to the solution of this particular situation.

According to the invention, sample portions of the two SAE steels mentioned are heated to temperatures at least equaling the highest of the lower heating critical temperatures of the two steels, this being the SAE 1035 steel having an  $Ac_1$  temperature of 1340 degrees F. The various portions are then cooled in a furnace maintained at a temperature lower than the highest of the lower cooling critical temperatures of the steels and at least equaling the lowest of the lower cooling critical temperatures of the two steels, this being the SAE 1335 steel having an  $Ar_1$  temperature of 1160 degrees F.

As soon as the portions cool to the temperature of this furnace, they are quenched and then tested to determine whether this quenching hardened them. Since the SAE 1335 steel has a lower cooling critical temperature less than that from which the portions are quenched, and the SAE 1035 steel has a higher lower cooling critical temperature, it follows that the former steel will be hardened while the latter will not. Therefore, testing of the various portions to determine whether they hardened during the quenching provides a means for determining their identities.

As the invention is now practiced, small sample pieces of the mixed stock of the two steels are heated in an ordinary rivet heating machine for approximately twenty seconds, which is sufficient to heat them to temperatures above the highest of the upper heating critical temperatures of the two steels, this being the SAE 1035 steel having an  $Ac_3$  temperature of 1475 degrees F. The pieces are then quickly placed in a muffle furnace maintained at approximately 1200 degrees F. for a sufficient length of time for the 50

pieces to reach this temperature, this normally taking only a few minutes, whereupon the pieces are quenched. Upon testing for hardness, the SAE 1035 steel will have a Brinell hardness in 5 the neighborhood of 160, while the SAE 1335 steel will run from 400 to 500. Obviously, this provides a very easy means for identifying the various pieces and for consequently permitting accurate rearrangement of the stock for better 10 storage or shipment.

Although the quenched pieces are described as being tested for Brinell hardness, it is possible to obtain reasonably accurate results by merely testing the quenched pieces with a file. In all 15 cases the mixed pieces of the different steels can be identified much more economically and rapidly than when the prior art procedure is resorted to.

I claim:

1. A method of determining the identities of 20 mixed pieces of SAE 1035 and SAE 1335 steels to permit their classification in separate groups, said method including heating sample portions of said pieces to temperatures above the highest of the upper critical temperatures of said steels, 25 cooling said portions in a furnace maintained at a temperature lower than said highest critical temperature and at least as high as the lowest critical temperature of said steels, quenching said portions, testing said portions to determine 30 whether they hardened during said quenching and classifying said pieces in separate groups according to whether said portions thereof were hardened.
2. A method of determining the identities of 35 mixed pieces of steels having different critical temperatures and of approximately the same carbon contents to permit their classification in separate groups, said method including heating sample portions of said pieces to temperatures 40 above the highest of the upper critical temperatures of said steels, cooling said portions in a furnace maintained at a temperature lower than said highest critical temperature and at least as high as the lowest critical temperature of said steels, quenching said portions, testing said portions to determine whether they hardened during 45 said quenching and classifying said pieces in separate groups according to whether said portions thereof were hardened.

HERBERT H. SCHNEIDER.